

July 6, 1943.

R. R. WEBSTER

2,323,695

METHOD OF CONTROLLING THE STRAIN-SENSITIVITY OF BESSEMER STEEL

Filed April 1, 1941

Fig. 1.



Fig. 2.



Fig. 3.



INVENTOR

Richard R. Webster

by his attorneys  
Stebbins and Blenko

## UNITED STATES PATENT OFFICE

2,323,695

METHOD OF CONTROLLING THE STRAIN-  
SENSITIVITY OF BESSEMER STEELRichard R. Webster, Beaver, Pa., assignor to Jones  
& Laughlin Steel Corporation, Pittsburgh, Pa.,  
a corporation of Pennsylvania

Application April 1, 1941, Serial No. 386,260

5 Claims. (Cl. 75—60)

This invention relates in general to the manufacture of Bessemer steel and, in particular, to the control of the strain-sensitivity thereof.

All steel exhibits a change in physical properties when subjected to cold working, i. e., deformation at a temperature below the recrystallization temperature. The change in physical properties is roughly proportional to the extent of the cold working but some steel exhibits a greater change than others for the same degree of cold working. The term "strain-sensitivity" designates the index of the rate of change of physical properties for a given amount of cold working.

The Graham et al. Patent No. 2,174,740 discloses a method of controlling the strain-sensitivity of steel by adjusting the proportion of oppositely effected nitrides contained therein. Iron nitrides increase the strain-sensitivity and aluminum nitride decreases it. In the Bessemer process of making steel, except for additions prior to pouring, the blown heat is substantially free from those nitrides such as aluminum nitride which reduces the strain-sensitivity. It is desirable, for certain purposes, to produce "rimmed" steel of low strain-sensitivity, but this cannot be produced by aluminum additions, because the addition of aluminum to reduce the strain-sensitivity "kills" the steel and thereby prevents "rimming" thereof.

I have discovered that I can effect a control of the strain-sensitivity similar to that obtained according to the practice of the Graham et al. patent with additions of iron or aluminum nitrides, by controlling the temperature at which a heat of iron is blown in the Bessemer converter. Even though the permissible range of the temperature of the metal during blowing is relatively narrow, I am able to obtain a considerable range of strain sensitivities in the finished steel. By my method of controlling the strain-sensitivity of Bessemer steel, I am able to produce rimmed steel having low strain-sensitivity as well as killed steel of like characteristics.

In a preferred practice of the invention, I control the amount of nitrides originally formed in the steel by the combination of the nitrogen in the air blast with the iron from which the steel is converted. I have discovered that, in steel containing no aluminum nitride, or similarly effective nitrides, the strain-sensitivity depends on the nitrogen content and that the amount of nitrogen from the air blast combining with the iron may be controlled within limits by varying the temperature at which the metal is blown. If a heat of Bessemer steel is blown at a relatively low temperature, such as 2925° F., the nitrogen content in the finished steel (in the form of iron nitride) is as low as

.008 percent or .007 percent. If the steel is blown at a higher temperature, e. g., 3040° F., the nitrogen content may be as high as .022 percent.

5 In practicing my invention, I depart from the normal Bessemer practice and control the temperature of the melt in order to obtain the desired nitrogen content and strain-sensitivity in the finished product. The temperature of the melt is preferably determined by the use of an optical pyrometer sighted on the metal. An indication of the temperature of the melt may also be obtained from the height of the curve drawn by the photometric recorder disclosed in Work

10 Patent No. 2,207,309. A further possible method of temperature determination is to subject a photo-cell to the radiation through the tuyères and record the current produced thereby.

15 Various methods of regulating the temperature of the melt during the blow in a Bessemer converter are known to the art. If the temperature of the melt is too high, it may be reduced by charging scrap or ore into the converter or by admitting steam to the air blast.

20 If the temperature of the bath is too low, it may be raised by "side-blowing," i. e., by tilting the converter so that some of the tuyères are uncovered.

25 The temperature of the melt may also be controlled by varying the temperature or composition of the iron charged into the converter. If the iron has a high silicon content, it will be heated to a higher temperature during the blowing, by the oxidation of the excess silicon, than if the silicon content is low. Ferro-silicon may even be added to the charge to increase the temperature rise of the melt during the blow. The temperature of the melt is similarly affected by the amount of carbon present in the iron. The 30 temperature at which the iron is charged into the converter may be varied somewhat and naturally has a direct effect on the temperature of the melt during the blow.

35 My invention is useful in the manufacture of steel by the duplex process, i. e., that in which the steel is first partially blown in a Bessemer converter and then further refined in an open-hearth furnace.

40 The accompanying drawing illustrates the use of the photometric apparatus of the aforementioned Work Patent No. 2,207,309 for indicating the temperature of the melt, and the strain-sensitivity characteristics of typical steels produced by my invention. In the drawings,

45 Figure 1 shows the variation of radiant-energy emission during the entire course of the blow of a melt whose temperature was determined by other means, such as an optical pyrometer, to be about 2990° F.

50 Figure 2 is a similar curve for the blow of a

melt whose temperature was about 3090° F.; and

Figure 3 is a set of curves showing the strain-sensitivity of two typical steels produced by my invention.

In conventional Bessemer practice, the blower usually attempts to maintain the melt at a temperature intermediate the permissible extremes, e. g., about 2970° F., with a preference for a somewhat higher temperature, in order to avoid any possibility of "skulling" in the converter. In practicing my invention, I blow the melt at a temperature considerably higher than 2970° F., e. g., as high as 3050° F., or at a temperature considerably lower than the 2970° F., e. g., 2930° F., depending on whether I desire to produce steel having high or low strain-sensitivity. Thus I deliberately approach either the temperature at which damage to the converter lining occurs or that at which "skulling" occurs in the converter, contrary to the usual practice, in order to obtain a product having the desired characteristics. The temperatures stated are those existing toward the end of the blow. In the early stages of the blow, i. e., prior to the removal of a substantial amount of carbon, the combination of nitrogen with iron is slight at any blowing temperature.

After the blow has proceeded to the point at which the desired removal of carbon has been obtained (see Work Patent No. 2,207,309), the temperature of the melt having been brought to the proper value toward the end of the blow by the known methods of control previously mentioned, the steel is poured from the converter in the known manner, in an aluminum-free condition and without the addition of any substantial amount of any other agent combining with nitrogen. After pouring, the steel is converted to usable form by the usual hot and cold working procedures.

Figure 2 shows the variation in the toughness (in resistance to the Izod impact test) of two steels of different nitrogen contents when subjected to increasing amounts of cold working. In other words, Figure 2 illustrates the relationship between the embrittlement of the steel and the degree of cold work to which it is subjected. These curves are obtained in the manner disclosed in the Graham et al. patent above mentioned. Curve A in Figure 2 is characteristic of Bessemer steel made according to my invention having a nitrogen content of about .008 percent. Curve B illustrates the strain-sensitivity characteristics of steel made according to my invention having a nitrogen content of about .020 percent.

It will be apparent from the foregoing description and explanation that the invention is characterized by important advantages over previous steel-making practices. In the first place, the invention makes it possible to produce rimmed Bessemer steel having a relatively low strain-sensitivity. The invention may be applied, furthermore, to the manufacture of killed steels which have been deoxidized with silicon or manganese but not aluminum.

Previous to my invention, there was no method known for controlling the absorption of nitrogen by the steel during the blow in a Bessemer converter. In ordinary Bessemer practice, variations in nitrogen contents from blow to blow of 50% or more are common with consequent variations in strain-sensitivity. This uncontrolled

variation has been largely responsible for the view that Bessemer steel is unreliable or even treacherous. By my invention, however, I am able to produce Bessemer steel which is uniform

5 from blow to blow in respect to its strain-sensitivity. As shown by the figures given above, the nitrogen content of the steel may be rather closely controlled, despite the fact that the permissible range of temperatures in blowing Bessemer steel is only from about 2900° F., at which temperature the full blown steel will begin to solidify, and the maximum of about 3150° F. to which the refractories lining the converter may safely be subjected. The figures already given 10 furnish a good example of the degree of control over the nitrogen content which I am enabled to achieve. The nitrogen content of Bessemer steel blown at 2930° F. is about .008 percent, while steel blown at a temperature of 3030° F. or above will have a nitrogen content of about .020 percent, i. e., 2.5 times the nitrogen content of steel blown at a temperature only 100° lower.

20 Although I have disclosed but a preferred practice of the invention, it will be apparent that changes in the procedure described may be made without departing from the spirit of the invention or the scope of the appended claims.

I claim:

1. In a method of controlling the strain-sensitivity of Bessemer steel, the steps including placing a heat of molten iron in a converter, blowing air therethrough, and adding scrap or ore to the heat during the blow to hold the temperature of the bath below about 2950° F., thereby producing a controlled nitrogen content in the steel at the conclusion of the blow.

2. In a method of controlling the strain-sensitivity of Bessemer steel, the steps including placing a heat of molten iron in a converter, blowing air therethrough, and introducing a cooling agent into the heat during the blow in an amount sufficient to hold the temperature of the bath below about 2950° F., thereby producing a controlled nitrogen content in the steel at the conclusion of the blow.

3. In a method of making Bessemer steel having a relatively low strain-sensitivity, the steps including placing a heat of molten iron in a converter, blowing air therethrough, and maintaining the temperature of the iron below about 2950° F. during the blow, thereby producing a controlled nitrogen content in the steel at the conclusion of the blow.

4. In a method of controlling the strain-sensitivity of Bessemer steel, the steps including placing a heat of molten iron in a converter, blowing air therethrough, introducing a cooling agent into the heat during the blow and thereby maintaining the temperature of the iron below 2950° F. during the blow so that the amount of the nitrogen of the air blast combining with the iron is below .015%.

5. In a method of controlling the strain-sensitivity of Bessemer steel, the steps including placing a heat of molten iron in a converter, blowing air therethrough, maintaining the iron substantially free from aluminum, introducing a cooling agent into the heat during the blow and thereby maintaining the temperature of the iron below 2950° F. during the blow so that the amount of the nitrogen of the air blast combining with the iron is below .015%.

RICHARD R. WEBSTER.